

Sept. 18, 1934.

D. ABERNETHY

1,974,228

GELATINOUS PRODUCT

Filed Sept. 29, 1931

FIG. 1.



FIG. 2.



FIG. 3.



Inventor

DAVID ABERNETHY

By *Sennies & Sennies*  
Attorney

## UNITED STATES PATENT OFFICE

1,974,228

## GELATINOUS PRODUCT

David Abernethy, Omaha, Nebr.

Application September 29, 1931, Serial No. 565,889

5 Claims. (Cl. 87—7)

This invention relates in general to glue and other gelatinous substances and more especially has reference to a gelatin product in such form that it may be rapidly dried and readily dissolved for use.

Glue and other gelatinous products, such as gelatin, which are prepared from animal matter, are extracted from the animal material in the form of a solution which is evaporated to the consistency of a jelly and is then dried to the form of glue which is available on the market. Considerable difficulties are encountered in drying the glue or other gelatinous material from the jelly-like mass to a hard, solid form in which it is known commercially. In drying, the conditions must be very closely regulated in order to effect the proper drying of the glue or other gelatinous material. Due to the fact that the drying of bodies of gelatinous material takes place at the surface exposed to the drying medium, the period for drying is prolonged. There is a tendency for the formation of a more or less impervious coating on the body of glue or other gelatinous material, which retards the drying. It will be appreciated, therefore, that if bodies of glue or similar material are subjected to this type of drying, the material to be dried must be exposed to the drying medium for a considerable period of time in order that the material be completely dried.

After the glue is dried and prepared in a marketable form, it will be found that considerable time must be expended in order to get the glue into a solution so that it may be used. Attempts have been made to reduce the time of dissolution, but even when the material is finely divided, a considerable time is necessary.

The present invention seeks to overcome the disadvantages inherent in the prior art by forming the glue jelly in bodies of such shape that the maximum amount of surface area is provided for the volume of glue. It has been found that by preparing the glue jelly in the form of small catkin-like bodies, the same may be rapidly dried upon exposing it to the action of a drying medium. Also, the finished product which is in the form of catkin-like bodies is readily soluble in water and may be very quickly prepared for use.

An object of this invention is to provide a gelatin product which may be rapidly dried.

Another object of this invention is to prepare a glue or other gelatinous product in such a form that the surface area of the product is relatively high compared to its volume.

Yet another object of this invention is to pre-

pare glue or other gelatinous substances in the form of porous bodies.

Still another object of this invention is to provide a glue or other gelatinous material product in the form of a catkin having air incorporated therein.

A still further object of this invention is to provide a gelatin-like product comprising gelatinous material in granular form having air incorporated therein and formed into catkin-like bodies.

With these and other objects in view which may appear incident to improvements herein set forth, the invention consists in the formation of glue or other gelatinous material in the form of bodies so shaped as to provide for the rapid drying of the same and the rapid dissolution of the dried product when the same is to be used.

In the drawing, there are shown several figures illustrating the form of the product prepared in accordance with the present invention.

In the drawing:

Figure 1 is a view of a mass of catkin-like bodies of gelatinous material prepared in accordance with the present invention.

Figure 2 is a close up view of a catkin of gelatinous material.

Figure 3 is a cross sectional view taken through one of the catkins of gelatinous material showing the manner in which air is incorporated in the granular gelatinous material.

In accordance with the present invention, glue or an edible gelatin is treated to form the same into small catkin-like bodies, the outer surface of which is covered with a multiplicity of spicules which tend to increase the ratio of the exposed surface area to the total volume of the bodies. It will be appreciated that such bodies may be more rapidly dried upon exposing them to a drying atmosphere than bodies in which the ratio of the surface area to the volume is low.

Since the rate of drying of glue or other gelatinous substance is a function of the ratio of the area to the volume, any body of the material in which the ratio of the surface area to the volume is relatively high, may be dried at a higher rate than bodies of the gelatinous material in which the surface-volume ratio is low.

Gelatinous products prepared as herein described have a relatively high surface-volume ratio, and consequently may be subjected to rapid drying without the disadvantage of producing bodies, the exterior of which is dry and the interior of which is in a soft moist condition.

In preparing the gelatin bodies having a high surface-volume ratio, steps must be taken to alter

the physical property of the material, so that it will retain its form while drying. It has been found that if the gelatinous material is reduced to a jelly like consistency and is then granulated 5 and intimately mixed with air, a mass will be obtained that will retain its form during drying.

If the gelatinous material is granulated and mixed with air under pressure, and then is extruded through small apertures, the mass will be 10 projected in the form of catkin-like strings having a multiplicity of spicules on its surface.

Upon extrusion of the catkin-like bodies through the small apertures, the mass of granulated gelatinous material having air incorporated 15 therein is expanded by reason of the release of pressure on the air incorporated in the granulated mass. This results in the production of bodies having an intumesced appearance and which are highly porous.

20 In the preparation of gelatinous products in accordance with the present invention, the solution containing the gelatinous material is evaporated to the desired specific gravity, which upon chilling, will result in the production of the more or less solid body. This solution is then run into 25 a trough which distributes the same in a thin layer upon a chilled roll. If the warm solution which is of jelly-like consistency is at a temperature between 110 and 120° F., and is deposited 30 as a thin film on the chilled roll, a solid film will be produced on the roll. It is preferable to regulate the temperature of the roll so as to cause the film of gelatinous material on the roll to be reduced to a temperature approximating 40° F. 35 This cooled film is scraped from the roll and the flakes resulting from the scraping of the film from the roll are then further treated to produce the desired product.

The successful production of the catkin-like 40 bodies of gelatinous material depends upon several conditions, namely, the amount of dry solids contained in the gelatinous solution after evaporation; the pressure in the chamber in which the material is mixed with air; and the temperature 45 in this chamber. In order to illustrate the possible variations in the process, it has been found that a medium grade or quality of glue may be treated in accordance with the present invention, if the solution is evaporated to produce a jelly of 50 14° Baumé, containing 31% dry solids and 69% water. In this instance, pressures from 50 to 70 pounds per square inch in the compression chamber work satisfactory. For a better grade of glue, the solution was evaporated to 10° Baumé, containing 55 21.5% dry solids and 78.5% water. In this instance, the pressure may range from 30 to 40 pounds per square inch. With a high grade of hide glue, ideal results may be obtained if the solution is evaporated to 7° Baumé, containing 60 14.5% dry solids and 85.5% water. In this instance, the pressure in the compression chamber may range from 20 to 30 pounds per square inch.

For the best operation, the temperature of the 65 jelly during the intermingling of the same with air should be maintained around 40° F. In this instance, satisfactory results are obtained if the temperature is maintained between 36 and 40° F.

As before pointed out, in order to produce the 70 product forming the subject matter of the present invention, it is necessary to granulate the gelatinous material and incorporate air therein. One method of accomplishing this result is to introduce the chilled flake jelly into a chamber in which is positioned a revolving screw. The revolving screw 75 is approximately the same diameter as the cham-

ber, and in addition to granulating the mass of flake jelly and incorporating air therein, the granulated aerated mixture is forced toward one end of the chamber. It is preferable to so construct the screw that it will have a tendency to beat or incorporate the air into the flake jelly. The mass of granulated aerated gelatinous material which is forced toward one end of the chamber by reason of the screw will be placed under a pressure. In order to produce the product forming the subject matter of the present invention, apertures are provided in the compression end of the chamber containing the mass of granulated gelatinous material and air under pressure, through which the mass is extruded into the atmosphere. Upon being extruded into the atmosphere, the mass tends to expand as a result of the pressure differential and the walls of the extruded mass burst through, forming a semi-porous light and fluffy catkin-like body of the gelatinous material.

80 In Figure 2 of the drawing, an enlarged view of the catkin-like body of extruded gelatinous material is shown. It will be noted from this figure that the outer surface of the string of material 1 is so serrated as to produce a plurality of small 85 spicules 2 which cover the entire surface of the catkin-like body.

90 In Figure 2 of the drawing, an enlarged view of the catkin-like body of extruded gelatinous material is shown. It will be noted from this figure that the outer surface of the string of material 1 is so serrated as to produce a plurality of small 95 spicules 2 which cover the entire surface of the catkin-like body.

As the mass of gelatinous material is extruded from the apertures in the wall of the compression chamber, there is a series of explosions resulting 100 in the formation of the spicules. As a result of the series of explosions, the catkin-like string of the material has the spicules rather evenly spaced along the surface of the material. In addition to the spicules formed upon the surface of the 105 catkin-like string of gelatinous material, the interior of the body is rendered porous by reason of the expansion of the air particles entrapped in the mass of the granulated material. In Figure 110 3, a cross section through the catkin-like string 115 illustrates the manner in which the air bubbles 3 are formed within the interior body of the string. In addition to the relatively large bubbles 3 shown in Figure 3, the entire body of the catkin-like 120 string of material is rendered porous by reason of the granulation of the glue jelly before the same is formed into the catkin. The spicules, of course, are porous to the same extent as the body of the 125 catkin-like string.

While the sponge-like spicules formed on the 130 surface of the explosion product extruded through the apertures in the pressure chamber have the appearance of spines on a catkin, they also are of 135 petticoat formation and somewhat resemble the form of so called petticoat insulators. It will be appreciated that as a result of the reduction in pressure upon the mass extruded through the apertures in the wall of the compression chamber, a product is obtained, the surface area of which is relatively high compared to the volume of the material. Also, as a result of the granulation of the same, and the incorporation of air therein, a porous product is obtained having a plurality of air voids therein.

In most instances, it has been found that as a 140 result of the incorporation of the air in the granulated mass of gelatinous material, its volume is increased approximately six times that of the original body of gelatinous material. Also, as a result of the production of the serrated surface on 145 the catkin-like body, the surface area is increased several hundred times that of the original surface area of the body of the glue.

The bodies of porous granular sponge-like structure extruded from the chamber of the mixing 150

device when deposited upon the conveyor belt for conveying the same into a dryer will retain their shape so as to permit drying of the material in substantially the same form as it is extruded from the pressure chamber.

It has been found from actual experiment that gelatinous material in the form produced as herein described may be dried in a period of approximately two hours compared to a matter of days in the drying of the ordinary glue products. Drying of the products herein described may be effected in any desired manner. For instance, the products may be deposited upon a porous conveyor belt which moves the material through the drying chamber in which the material is subjected to the action of a drying gas. Of course, other methods of drying may be resorted to to effect drying of the product.

After the product is dried, it will be found that the same is in the form of catkin-like strings of porous sponge-like materials, the outer surface of which is covered with a plurality of petticoat-like spicules. The high surface-volume ratio of the product extruded from the compression chamber still exists in the finished dry product. This property is advantageous in the finished product in water. In the case of glue, such as property is highly advantageous in that the glue may be rapidly prepared for use in a minimum of time. For instance, glue prepared in this form can be soaked in cold water and be ready for joint work in thirty minutes. The glues prepared in accordance with prior art methods require from ten to twelve hours to effect a solution of the same, even when ground relatively fine.

In addition to the products shown in the drawing, the material may be extruded from the compression chamber in tubular form, in which instance, the catkin-like strings will be relatively hollow, affording a larger surface area. It is also within the purview of my invention to form the material into a flat band, or any extruded shape continuously formed.

45

50

55

60

65

70

75

While the present product has been described with particular reference to glue, it is to be clearly understood that products having the form herein described may be prepared from glue, edible gelatin or other gelatinous materials.

While I have shown and described the preferred embodiment of my invention, I wish it to be understood that I do not confine myself to the precise details herein set forth by way of illustration, as it is apparent that changes and variations may be made by those skilled in the art without departing from the spirit of the invention, or exceeding the scope of the appended claims.

I claim:

1. A dry glue product having a large surface ratio and in the form of a string-like unit having a plurality of substantially overlapping and nested petticoat serrations extending from a central axis.

2. A dry spongelike glue product having a large surface ratio and in the form of a string-like unit having a plurality of substantially overlapping and nested petticoat serrations extending from a central axis, such serrations being formed by 100 planes of cleavage.

3. A dry, granulated and spongelike glue product in the form of a string-like unit having a plurality of substantially overlapping and nested petticoat serrations.

4. A dry, granulated and spongelike glue product in the form of a string-like unit having a plurality of substantially overlapping and nested petticoat serrations extending from a central axis.

5. A dry, granulated and spongelike glue product in the form of a string having a plurality of substantially overlapping and nested petticoat serrations extending from a central axis, such serrations being formed by planes of cleavage.

DAVID ABERNETHY.

80

85

90

95

105

110

115

120

125

130

135

140

145

150